

June 11, 1940.

M. W. DITTO

2,203,778

METHOD FOR PRODUCING STEEL

Filed July 11, 1939

3 Sheets-Sheet 1

Fig. 1.



Inventor

M. W. Ditto,

By Seymour, Bright & Nottingham

Attorneys

June 11, 1940.

M. W. DITTO

2,203,778

METHOD FOR PRODUCING STEEL

Filed July 11, 1939.

3 Sheets-Sheet 2.

Fig. 2.



Fig. 3.



Inventor

M. W. Ditto,

By Seymour, Brights Nottingham

Attorneys

June 11, 1940.

M. W. DITTO

2,203,778

METHOD FOR PRODUCING STEEL

Filed July 11, 1939

3 Sheets-Sheet 3



Inventor  
M. W. Ditto,  
Seymour, Bright  
& Nottingham

Attorneys

## UNITED STATES PATENT OFFICE

2,203,778

## METHOD FOR PRODUCING STEEL

Marvin W. Ditto, New York, N. Y., assignor to  
 Emulsions Process Corporation, New York,  
 N. Y., a corporation of Delaware

Application July 11, 1939, Serial No. 283,902

16 Claims. (Cl. 75—60)

This invention relates to an improved method for producing steel in metallurgical furnaces, and more particularly to the production of steel in a Bessemer converter or furnace.

5 In using a Bessemer converter, it is well known that molten pig iron or cast iron is poured into the furnace and a blast of air is turned on and introduced into the molten metal. Each ton of pig iron contains about 75 pounds of carbon, 25 10 pounds of silicon, 1 pound of sulphur, and 15 pounds of manganese, most of which will be burned out. These elements are ordinarily the fuel. The molten iron is at a temperature of about 2200° F. when poured into the converter. 15 In a few minutes after the blast of air is turned on, the burning of these elements in the iron raises the temperature of the charge to about 3500° F. Most of the carbon, silicon, sulphur and manganese are burned out, and ordinarily, 20 no external fuel is necessary.

When the impurities are burned out, the correct amount of carbon and manganese may be added to give the steel the final composition desired. The steel is then poured from the converter into ingots ready to be made into shapes 25 suitable for use.

I have discovered that such method is improved by adding to the air blast the products of dissociation and combustion resulting from the 30 burning of a water-in-fuel oil emulsion or its equivalent during the blast period.

Due to my improvements, the total air introduced into the furnace is preheated and the water in the emulsion is raised to the flame temperature of the burning fuel. Consequently, the 35 water vapor entering into reaction with the carbon of the fuel oil is dissociated into carbon monoxide and hydrogen. As a result of introducing a gas rich in oxygen, (resulting from the further 40 dissociation of the water vapor by contact with the molten iron in the furnace), the FeO rate of formation is increased. The water being a relatively rich bearer of oxygen, reduces the amount of atmospheric oxygen required, therefore, by my process, the amount of nitrogen introduced into the furnace is reduced. By regulating the amount of fuel introduced into the 45 blast air, it is possible to increase and maintain the temperature of the metal after normal reactions have taken place. As a result of a larger 50 amount of oxygen available and the large amount of hydrogen present, the rate of sulphur reduction is increased, and a larger percentage of sulphur is gasified and eliminated from the molten metal.

By introducing hydrated lime into the emulsion, a larger percentage of phosphorus can be eliminated by the reaction with the calcium. Irons running higher in phosphorus than are normally used in Bessemer practice are made 5 available by my procedure.

Furthermore, in accordance with my invention, I can govern the moisture content of the blast air used in the furnace, and this can be accomplished by increasing or decreasing the 10 amount of water in the emulsion in accordance with the moisture content of the blast air. For example, in winter time, the relative humidity of the blast air may be as low as 10%, and at such times I will increase the amount of water forming part of the emulsion. On the other hand, in the summertime, the humidity may be as high as 95%, and at such times, I will decrease the amount of water incorporated in the emulsion. 15

Having now indicated in a general way the 20 nature and purpose of my invention, I will proceed to a detail description thereof, with reference to the accompanying drawings, in which I have illustrated a preferred embodiment, and in which:

Fig. 1 is a vertical sectional view of a portion of a Bessemer converter modified to accord with my invention.

Fig. 2 is a view similar to Fig. 1, but taken on the line 2—2 of that figure.

Fig. 3 is a horizontal sectional view taken on the line 3—3 of Fig. 2.

Fig. 4 is a flow diagram showing the converter hooked up with the means for supplying a water-in-fuel oil emulsion to the converter.

Referring to the drawings, 6 designates a Bessemer converter having a shell 7, a base ring 8, hanger bolts 9, bottom shell 10, refractory lining 11, tuyère blocks 12, tuyères 13, tuyère block supporting ring 14, combustion arch 15, refractory bottom shell lining 16, wind duct 17, burner opening 18, atomizing nozzle 19, fixed emulsion conveying header 20, flexible emulsion conveying tube 21, trunnions 22, air supply conduit 23, main air supply pipe 24, trunnion supports 25, worm tilting gear 26, reduction gear 27, motor 28, and tangential air ports 29.

So far as the converter is concerned, all of the parts, with the exception of 18, 19, 20 and 21, are of more or less conventional construction, 50 and the motor 28 is employed in the usual way to operate the gearing to cause the converter to move from a vertical position to a horizontal one, and vice versa.

Referring now to the flow sheet in Fig. 4, it 55

- will be noted that fuel oil is introduced through a pipe 30 into a preheater 31 which may be heated by any suitable means. For example, steam may be introduced into the preheater through a pipe 32 and be discharged through a pipe 33. The preheated oil is passed through a pipe 34 into one end of a proportioning pump 35, preferably of a type to permit variation of the proportions of liquids pumped while the pump is in operation.
- 10 A good example of such a pump is disclosed in my application Serial No. 230,480, filed September 17, 1938, although I can accomplish the same purpose by employing a pair of pumps of the type illustrated in the U. S. patent to Fenchelle, No. 1,289,716.

The hot oil is forced by such a pump structure at high superatmospheric pressure through a pipe 36 into a manifold 37 that leads to a motor driven emulsifying mill 38 which may be of the kind disclosed in the Russell U. S. Patent No. 2,059,535, but is preferably of the type disclosed in my application Serial No. 218,883, filed June 12, 1938. Water which may be preheated, is fed to the opposite end of the proportioning pump through a conduit 39 having a control valve 40, and the water is forced under high superatmospheric pressure from the pump through a pipe 41 into the manifold 37 where it may be mixed with the hot oil before the mixture is introduced into the inlet of the emulsifying mill. In the latter, the water and oil are incorporated into a relatively stable water-in-fuel oil emulsion, and the hot emulsion, due to the pressure imparted to the liquids by the pump 35, is forced through a pipe 41a into an emulsion heater 42 where the temperature of the emulsion may be raised to any desired degree by superheated steam or the like. The steam is introduced at 43 and discharged at 44. The highly heated emulsion is passed from the heater 42 through a pipe 45 into the header 20, from which it may be passed through the flexible tube 21 to the nozzle 19 of the converter.

In practicing the process, the emulsifying mixer or dispersion mill 35 converts the oil and water

45 into an oil phase emulsion, and this emulsion, in heated condition, is fed to the nozzle 19.

In practice, the blast air for the converter is passed through pipe 24, conduit 23, wind duct 17, and tangential ports 29, into the combustion chamber 46 of the converter, and due to the tangential ports, it is given a whirling motion. This air being under a pressure of approximately 25 to 40 pounds per square inch, is turned into the furnace when the latter is in a horizontal position for reception of the molten pig iron charge. As the furnace is tilted back into vertical position, the pressure of the air passing through the tuyères 13 prevents the hot metal from gravitating through the tuyères, and the air passes upwardly into intimate contact with the metal during the blow period. Simultaneously, when the air blast is turned on, the valve (not shown) controlling the supply of hot emulsion, is opened, and the emulsion is introduced into the combustion chamber 46 and ignited, and combustion takes place under the pressure conditions existing in this chamber. This results in an intense rate of combustion, due to the fact that the burner 19 is at the center of the vortex of the whirling currents of air.

I have found that the ignitability and combustibility of the emulsion can be maintained with as much as 50% of water being incorporated into the fuel oil, and that upon combustion, the water impounded in the emulsion is immediately

raised to the temperature of the flame. At these temperatures, part of the water reacts with the carbon to form carbon monoxide and hydrogen gas; these products, including the water vapor resulting from excess water not entering into the reaction, are forced by the air stream through the tuyère blocks and into the metal at the base of the furnace. The highly heated water vapor when brought in contact with the hot metal, reacts with iron to form FeO and hydrogen. Also, it will enter into reaction with the manganese of the molten pool to form MnO and hydrogen, and also will enter into reaction with the sulphur to form SO<sub>2</sub> and hydrogen. (Some of the sulphur will enter into reaction with hydrogen to form hydrogen sulphide.)

Under conventional operating conditions as used in Bessemer converters today, it is assumed that the oxygen obtained from the atmosphere first oxidizes the silicon into silica. The manganese then enters into reaction to form MnO, and then the carbon enters into reaction to form carbon monoxide and carbon dioxide. It is assumed that the larger part of the carbon content of the iron is oxidized as a result of reaction between the carbon and FeO resulting in the following reaction: FeO plus carbon equals Fe and CO.

As water contains a larger percentage of oxygen than atmospheric air per pound by weight, by this means of introducing water into the converter, a gas rich in oxygen is introduced, and it eliminates the necessity of supplying all the oxygen from the atmosphere.

One objection to Bessemer steel has been the large amount of iron nitride formed as a result of high temperature, and the combination of iron with nitrogen in the atmosphere. By enriching the air with oxygen from the water, a large percentage of nitrogen is kept out of the furnace, therefore there is less tendency to combine with nitrogen to form the objectionable nitrides.

Pig iron running high in phosphorus can be reduced to the minimum by the addition of hydrated lime to the water. Such hydrated calcium may be introduced into the pipe 39 through a valved pipe 50. By my apparatus, it is possible to introduce this lime in a finely divided state into the metal bath, and intimately disperse the same throughout the molten metal. Therefore, the slag resulting from oxidation of silicon segregates the impurities and will contain the lime and phosphorus in the form of calcium phosphate. The phosphorus will then be carried out of the converter with the slag.

By the means disclosed herein, a better quality of Bessemer steel can be obtained, and by the control of the percentage of water introduced into the converter, better control of operating conditions is made available.

Reverting to the control of the percentage of water, it will be noted that this can be accomplished by means of the valve 40, and I prefer to control such valve by any suitable means responsive to movements of any preferred type of hygrometer 40a, as this will enable me to control the moisture content of the air in the combustion chamber 46. A suitable hygrostatic controller is shown in the patent to Grisby, No. 1,219,390, March 13, 1917. By such apparatus, as the relative humidity of the blast air increases, the hygrometer will cause partial closing of the valve 40 so as to reduce the volume of water incorporated into the emulsion. If, for best operating conditions it was found that the relative humidity

of the air, so far as furnace conditions are concerned, should be the maximum natural saturation of the air, I can incorporate enough water in the emulsion so that regardless of humidity 5 conditions in the winter time, with reduced atmospheric temperatures, the water content of the air passing through the furnace would be approximately the same as the water content conditions during the maximum humidity saturation 10 in the warm weather of summertime.

By my procedure I can always incorporate into the emulsion more than enough fuel oil to supply the necessary heat to the water so that there will be no heat demand upon the furnace conditions 15 to take care of the water passing through the furnace, as the temperature of the products of combustion of the emulsion can be raised to approximately the temperature of the flame at or adjacent to the tuyères, so that they can immediately enter into reaction with the other 20 products of the furnace.

Also by my improved procedure, I can not only condition the air employed in a Bessemer furnace, but can control the moisture content of the air 25 introduced into any type of metallurgical furnace which would be benefited by maintaining a uniform atmospheric condition within the furnace at all times. In other words, I believe, operating under such conditions, that practically all types 30 of furnaces, where control of water vapor is beneficial, such as open hearth, blast, cement kilns, lime kilns, enameling and japanning furnaces will be benefited by my method of operation.

While I have disclosed what I now consider 35 to be preferred modes of procedure, it will be understood that changes may be made in the details disclosed, without departing from the spirit of the invention, as expressed in the claims.

What I claim and desire to secure by Letters 40 Patent is:

1. In the production of steel in a Bessemer converter, introducing blast air into the lower portion of a pool of molten pig iron, simultaneously introducing into said air an intimate mixture of water and fuel oil in atomized condition, and burning such mixture in intimate contact with the air as the latter enters the molten pig 45 iron.

2. In the conversion of ferric metal high in 50 carbon into steel in the presence of atmospheric air, introducing into the bottom of a pool of such molten metal an intimate mixture of water and fuel oil in atomized condition, and burning such mixture in intimate contact with the air as the latter contacts with the molten metal, and thereby forming ferric oxides.

3. In the production of steel in a Bessemer converter, introducing blast air into the lower portion of a pool of molten pig iron, simultaneously 60 introducing into said air an emulsified fuel having water as a component thereof, and burning such fuel in intimate contact with the air as the latter enters the molten pig iron.

4. In the conversion of ferric metal high in 65 carbon into steel in the presence of atmospheric air, preheating an intimate mixture of water and fuel oil, and then introducing such mixture in atomized condition into said air, and burning such mixture in intimate contact with the air as the latter enters the bottom of a pool of the metal 70 while the metal is in molten condition.

5. In the production of steel in a Bessemer converter, introducing blast air into the lower portion 75 of a pool of molten pig iron, simultaneously introducing in said air a highly heated intimate mix-

ture of water and fuel oil in atomized condition, and burning such mixture in intimate contact with the air as the latter enters the molten pig iron.

6. In the production of steel in a Bessemer 5 converter, organizing blast air into a whirling current and passing such current into the lower portion of a pool of molten pig iron, simultaneously introducing into said current of air an intimate mixture of water and fuel oil in atomized 10 condition, and burning such mixture in intimate contact with the air as the latter enters the molten pig iron.

7. In the conversion of ferric metal high in 15 carbon into steel, forming a pool of such metal in molten condition, organizing a stream of blast air into a whirling current and introducing such air into the bottom of the pool, simultaneously introducing into the vortex of the air current an intimate mixture of water and fuel oil in atomized 20 condition, and burning such mixture in intimate contact with the air as the latter enters the bottom of the molten pool.

8. In the production of steel in a Bessemer 25 converter, introducing blast air into the lower portion of a pool of molten pig iron, simultaneously introducing into said air an intimate mixture of water, fuel oil and lime, and burning such fuel oil in contact with the air as the latter enters the molten pig iron.

9. In the conversion of ferric metal high in 30 carbon into steel in the presence of blast air, introducing an emulsified fuel having water as a component thereof into said air as the latter enters the bottom of a molten pool of such metal, and burning said fuel in intimate contact with the air as the latter enters the molten pool.

10. In the operation of a furnace utilizing atmospheric air, maintaining the moisture content 35 of the air within predetermined limits by introducing into the air an intimate mixture of water and fuel oil in atomized condition, burning such mixture in intimate contact with the air, and varying the water content of the mixture to accord with the moisture content of the air.

11. In the conversion of ferric metal high in 40 carbon into steel in the presence of blast air, introducing into said air an intimate mixture of water and fuel oil in atomized condition, and maintaining the moisture content of the air within 45 predetermined limits by increasing the water content of the mixture as the moisture content of the air decreases, and decreasing the water content of the mixture as the moisture content of the air increases.

12. In the conversion of ferric metal high in 50 carbon into steel in the presence of blast air, introducing into said air an intimate mixture of water and fuel oil in atomized condition and maintaining the moisture content of the air 55 within predetermined limits by increasing the water content of the mixture as the moisture content of the air decreases, and decreasing the water content of the mixture as the moisture content of the air increases, and burning said mixture in intimate contact with the air as the latter contacts such metal while the latter is in molten condition.

13. In the production of steel in a Bessemer 60 converter, introducing blast air into the lower portion of a pool of molten pig iron, simultaneously 65 introducing into said air an intimate mixture of water and fuel oil in atomized condition, maintaining the moisture content of said air within predetermined limits by varying the wa- 70

ter content of the mixture, and burning such mixture in intimate contact with the air as the latter enters the molten pig iron.

14. In the production of steel in a Bessemer converter, introducing blast air into the lower portion of a pool of molten pig iron, simultaneously introducing into said air an emulsified fuel having water as a component thereof, maintaining the moisture content of the air within predetermined limits by varying the water content of the emulsified fuel, and burning such emulsified fuel in intimate contact with the air as the latter enters the molten pig iron.

15. In the conversion of ferric metal high in carbon into steel in the presence of blast air, introducing into said air an intimate mixture of water and fuel oil in atomized condition, main-

taining the water content of the mixture at a predetermined degree to accord with the moisture content of the air, and burning such mixture in intimate contact with the air as the latter is contacted with the metal while the metal is in molten 5 condition.

16. In the production of steel in a Bessemer converter, introducing blast air into the lower portion of a pool of molten pig iron, simultaneously introducing into said air an intimate mixture of water and fuel oil in atomized condition, 10 maintaining the water content of the mixture at a predetermined degree to accord with the moisture content of the blast air, and burning such mixture in intimate contact with the air as the 15 latter enters the molten pig iron.

MARVIN W. DITTO.